

# UNITED STATES PATENT OFFICE.

CHARLES E. NELSON, OF CAPAC, MICHIGAN, ASSIGNOR TO EDWARD P. METCALF, OF PROVIDENCE, RHODE ISLAND, AND ADOLPH LOEWENTHAL AND CLIFFORD E. DUNN, TRUSTEES, OF NEW YORK, N. Y.

## PROCESS OF PRODUCING PAPER OR PAPER-BOARD AND THE LIKE

No. 879,888.

Specification of Letters Patent.

Patented Feb. 25, 1908.

Application filed February 23, 1907. Serial No. 358,774.

*To all whom it may concern:*

Be it known that I, CHARLES E. NELSON, a citizen of the United States, residing in Capac, county of St. Clair, and State of Michigan, have invented certain new and useful Improvements in Processes of Producing Paper or Paper-Board and the Like, of which the following is a full, clear, and exact specification.

10 This invention relates to a process of forming paper or board and the like from half-stuff containing peat fibers and the natural gelatinous matter of the peat.

The half-stuff containing peat fibers and 15 the gelatinous matter of the peat may be produced in any desired manner, as the production thereof does not form an essential part of the present invention. For instance half-stuff produced in the manner 20 described and claimed in U. S. Patent No. 836,069 granted November 13, 1906 on an application of Christian Esser, may be used, although the present invention is not to be confined to the use of the particular half-stuff 25 of the above patent, but may be employed with half-stuff containing peat fibers and the non-coagulated natural gelatinous matter of the peat, however produced.

The present process of producing paper or 30 board and the like from half-stuff containing peat fibers and gelatinous matter is designed to utilize not only the peat fibers, but also a considerable amount of the natural gelatinous matter of peat, and in the finished 35 product of the process the peat fibers give strength and body to the product, while comparatively large quantities of the gelatinous matter are present, adhering to the fibers and binding them together.

40 In carrying out the process of the present invention, the half - stuff containing peat fibers and gelatinous matter is supplied with a sufficient quantity of water or other liquid to float it, and is carried to the stuff chest.

45 From the stuff chest, the floated matter is conducted through the necessary screens to the machine cylinder tanks where the operation of converting it into paper, or board and the like is started. Prior to the actual

50 operation of making the half-stuff into paper board and the like, the fibers and gelatinous matter are subjected to the action of heat of such temperature that the gelatinous matter is softened sufficiently to destroy any

lumps which it may contain. This softening of the gelatinous matter by the action of heat brings it into a fluidic or soluble condition and causes it to be evenly and uniformly distributed among the peat fibers. Furthermore, by distributing the gelatinous matter uniformly among the peat fibers it will be obvious that the gelatinous matter will also be uniformly distributed throughout the paper board and the like when manufactured and will thus serve to render the finished product uniformly water-repellent and strong. The heating of the half-stuff prior to the operation of making it into paper board and the like, preferably is effected in the machine cylinder tanks, although if desired the heating may take place in the stuff chest.

In subjecting the gelatinous matter to the action of heat of such temperature that said matter will be softened sufficiently to destroy any lumps which it may contain, it must be borne in mind that the temperature must not be sufficient to cause coagulation of said gelatinous matter, which is albuminous in its nature.

55 After the floated half-stuff has been sufficiently heated to reduce any lumps in the gelatinous matter and to distribute the same evenly among the peat fibers, both the fibers and a comparatively large amount of the gelatinous matter are run into paper or board and the like.

60 It will be apparent from the above, that the finished product of the process contains peat fibers, together with a quantity of the gelatinous matter of peat, which latter acts 65 as a binder for the fibers.

If desired the half-stuff containing peat fibers and the natural gelatinous matter of the peat may have mixed therewith a small percentage of sulfid or other hard stock.

The board produced according to the present process possesses the desirable qualities of strength and durability and in addition is moth and vermin-proof; furthermore it is 70 damp-repellent even if unsized, and is also a non-conductor of electricity and an excellent insulating material.

75 The herein-described method of producing paper or board and the like from half-stuff containing peat fibers and the natural gelatinous matter of the peat by floating and heating the fibers and gelatinous matter of

the peat and then running both the fibers and gelatinous matter into paper board and the like may be varied widely, providing the consideration of maintaining a comparatively large quantity of gelatinous matter in connection with the peat fibers be kept in view.

What is claimed is—

1. A process of producing paper or board and the like from half-stuff containing peat fibers and the natural gelatinous matter of the peat, which process consists in heating the gelatinous matter insufficiently to coagulate the same, and running said gelatinous matter and the peat fibers into paper or board and the like.
2. A process of producing paper or board and the like from half-stuff containing peat fibers and the natural gelatinous matter of the peat, which process consists in floating and heating the peat fibers and gelatinous

matter insufficiently to coagulate said gelatinous matter, and then running said fibers and gelatinous matter into paper or board and the like.

3. A process of producing paper or board and the like from half-stuff containing peat fibers and the natural gelatinous matter of the peat, which process consists in heating the half-stuff to a temperature insufficient to coagulate the gelatinous matter, and then running the said half-stuff into paper or board and the like.

In testimony whereof, I have hereunto set my hand in the presence of two subscribing witnesses.

CHARLES E. NELSON.

Witnesses:

CLEMENT F. SISSON,  
O. A. PREY.